

## UNITED STATES PATENT OFFICE

RENE CLAVEL, OF BASEL, SWITZERLAND

## WEIGHTING NATURAL SILK

No Drawing. Application filed May 16, 1927, Serial No. 191,941, and in Germany September 17, 1928.

This invention relates to a method of weighting natural silk with metallic compounds.

Hitherto, in processes for weighting silk, a number of substances have been brought into contact with the fibre, but in separate baths, each containing only one weighting substance, and between each of the baths the silk has been thoroughly washed, acidified and neutralized. In practice the mineral weighting process has been used, with solutions of metal salts, more especially salts of tin. In this process the silk is first treated with a solution of chloride of tin at the usual 10 temperature for rather a long time, say for about an hour or two, and then thoroughly washed with water, in order to hydrolyze the tin-salts on the fibre. The precipitated stannic acid is then fixed by treating the 15 silk with a solution of di-sodium phosphate of about 6 per cent. strength, at a temperature of about 60° C. The tin-salts and phosphate treatments are repeated alternately until the desired weighting has been obtained, and after each bath the silk must 20 undergo a thorough washing or neutralization. After the last phosphate bath the silk may be treated with a solution of sulphate of alumina, and, after subsequent washing, with 25 a solution of water glass at a temperature of about 50° C. The silk which has been treated in this manner, and weighted with complex compounds of tin, phosphate and water glass, is then washed with soap, rinsed and soured. 30 The method of weighting which is described above, as well as other methods of weighting with various substances, wastes much time, on account of the number of baths, and the washing, acidification or neutralization which is necessary between each 35 bath. Such methods are also very expensive, and their disadvantages are not to be overcome by the use of the modern weighting centrifuges. The greatest of these disadvantages is the serious loss of material 40 which is caused by the many washing and neutralization processes, and the troublesome and expensive processes which are necessary for the recovery of the weighting substances from the waste liquors. 45

According to the invention the weighting of natural silk is considerably simplified and less expensive, when care is taken that the metal salts come in contact with the silk only at a certain high acid concentration or in 55 other words that the metal salts are acting upon the silk only in the presence of acids or acid salts. The acids or acid salts necessary for obtaining the high acid concentration may be added to the metal salt bath for 60 example a tin tetrachloride solution or the silk may be treated with acids or acid salts before taking it into the metal salt bath. The natural silk treated in such a manner with metal salts may then be brought with 65 out previous washing if desired after squeezing for removal of the excess of tin tetrachloride solution into the following phosphate bath. Due to the high acid concentration present during the metal salt treatment, the silk undergoes a change and the 70 tin chloride probably forms a compound with the silk, in which it is hydrolyzed. However, in no case undesired precipitations take place in the phosphate bath and the tin salt 75 on the fibre combines with the phosphate into a tin-phosphate compound, probably  $\text{Sn}(\text{HPO}_4)_2$ , adapted and necessary for weighting silk.

When treating silk with a tin chloride 80 solution without the presence of acids or acid salts it is not possible to bring the silk treated with the metal salts into the following phosphate bath without previous washing of the silk, to hydrolyze the tin chloride. There 85 would occur in the phosphate bath and upon the silk precipitations of tin salts which are not adapted for weighting purposes, make the silk turbid, cloudy and milky and produce spots. If one uses, however, in accordance 90 with the invention tin salt baths with increased acid concentration, undesired precipitations do not occur, the silk is abundantly weighed, looks unobjectionable, and shows no 95 spots.

In order to prevent the silk from being attacked too much by the increased acid concentration it is advisable to use protective colloids such as glue, gelatine, albumin or the like. These protective colloids may be 100

brought upon the silk either before bringing it into the acid tin salt solution for example by coating or impregnation if desired together with the acid substances, for example acids, or may be added to the tin salt bath. It is also possible to treat the silk before bringing it into the metal salt bath with acid substances such as acids or acid salts and to make this pretreatment in presence of protective colloids. The acid concentration may then be kept lower in the metal salt bath or the addition of acids or acid salts may be renounced. Also in these cases a change of the silk fibres takes place, which produces a more intensive and more equal taking up of the weighting means. Experiments show the surprising fact, that silks of different origin took up equal amounts of weighting substances. The weighting of the silk is then carried through by passing the silk through one or only a few weighting baths, in which the skeins or textures only had to remain a short time, to become sufficiently weighted.

A further development of the idea of my invention, namely the metal salt treatment in the presence of acid or acid salts, consists in that several of the weighting substances for example tin chloride and phosphate are applied together in one single bath, which has obtained increased acid concentration by the addition of acids or acid salts. Here too the weighting is carried through unobjectionably and no precipitations of undesired and unsuitable tin compounds take place, because the bath has an increased acid concentration. In this case it is advisable to use instead of phosphates, phosphoric acid, which serves a double purpose namely to produce the tin-phosphate compound and to increase the acid concentration. Here too the addition of protective colloids is advisable, because they do not only protect the silk but also help in preventing the precipitation of unsuitable tin compounds. It is even possible to add solutions of water glass, which is a substance used in the tin weighting process, to the weighting bath containing tin salt and phosphate at increased acid concentration, thus carrying the entire weighting process through with a single bath.

If one treats the silk with weighting baths according to the present invention, using proper concentration of the bath and a suitable temperature, the silk is sufficiently weighted after only a very short treatment. The precipitation reactions which are necessary for perfect weighting and cannot occur in the bath on account of the high acid concentration, or the presence of the protective colloids, if desired at high acid concentration, occur on the fibre immediately. It is therefore possible to produce weightings, which are satisfactory and of good quality by a simple application of the solution, such as by

drawing the skeins of silk material through the bath, or by dipping it into the bath.

In order to obtain a better fixing of the weighting substance, and in certain cases in order to remove the excess acid, it is advisable to put the silk into a press for freeing it of any liquid which adheres to it on removal from the weighting bath, and before drying to subject it to a bath having alkaline reaction. This after-treatment bath, consisting for example of a solution of ammonium carbonate, can if required also contain dyestuffs which contain tanning substances, such as haematein.

The following examples illustrate the invention:

*Example 1.*—Silk fabrics which have not been boiled off are placed on a finishing machine and drawn for example three times through a solution containing the following ingredients: 5 litres of tetrachloride of tin of 30° Baumé  $\frac{1}{2}$  litre of concentrated ortho-phosphoric acid and 1 litre of a solution of aluminum sulphate of 10 per cent strength.

The weighting is completed by a subsequent treatment at a temperature of 60° C. with solution of water glass of 4° Baumé.

*Example 2.*—The weighting bath contains the following ingredients: 6 litres of solution of tetrachloride of tin of 22° Baumé, 1 litre of concentrated formic acid, 1 litre of neutral solution of water glass of 4° Baumé, 120 grams of sodium phosphate, together with 100 grams of glue dissolved in 2 litres of water.

Boiled off silk after treatment in this weighting bath is pressed, drawn through a solution of ammonium carbonate of 10 per cent strength, and dried. The silk is washed in a soap bath to which haematein has been added, and then dyed.

*Example 3.*—A crêpe de Chine texture, consisting of natural silk is drawn in full breadth through a 1% solution of phosphoric acid containing 12 gr. glue per litre. The piece is then drawn through 4 tin chloride baths containing tin tetrachloride solution of 35° Bé. The piece then passes a squeezer and enters first a 10% mono-sodium phosphate bath and then a 6% bi-sodium phosphate bath. After the passage of the alkaline phosphate bath the silk goes through a hydro-extractor and is finished in half an hour in a water glass solution of at least 1° Bé. at 60° C. which contains 1 gr. soap per litre.

*Example 4.*—Silk skeins are dipped for a short time into a 10% solution of mono-chloroacetic acid. One lets the skeins drain and brings them then into a tin tetrachloride bath of 35° Bé. The skeins are dipped into this metal salt bath for a short time, drawn out again and left in the air for a short time. This process is repeated if necessary several times. The skeins are then carefully hydro-extracted and brought for a short time into

a 15% mono-sodium phosphate solution. After squeezing or hydro-extraction of the liquid if desired after washing, the skeins are finished by a short treatment in a soap containing water glass solution of at least 1° Bé, at 40° C.

Silk which is weighted in accordance with this invention does not lose in elasticity or strength and has full brilliancy. Owing to 10 the short treatment in the baths containing several weighting agents the appearance of the silk is considerably improved. The economical advantages of the new process are extraordinarily great, the number of weighting 15 baths is as far as possible reduced to a minimum, the washing and neutralization after each bath is rendered superfluous, and the transport of the silk from one bath to another is avoided. A further advantage consists 20 in the fact that owing to the elimination of the washing, acidifying and neutralization, there are not obtained diluted solutions of the weighting substances, or of the transformed products produced by the neutralization, the recovery of which substances 25 or products entails considerable expense and special installations.

A further advantage of the invention is that when weighting in the piece on the usual 30 finishing machine, the piece can be drawn through the solutions stretched to their full width, either singly or superimposed on each other, and in this manner the troublesome creases and spots on the silks which often 35 arise in consequence of the washing not having been properly carried out, or other defects, are avoided.

I claim:

1. A method of weighting natural silk 40 which comprises the steps of treating the silk successively with solutions of acid compounds, aqueous solutions of heavy metal compounds, and aqueous solutions of precipitating agents for the heavy metal compounds taken up by the silk.

2. A method of weighting natural silk 45 which comprises the steps of treating the silk successively with solutions of acid compounds, aqueous solutions of heavy metal compounds containing acid compounds, and aqueous solutions of precipitating agents for the heavy metal compounds taken up by the silk.

3. A method of weighting natural silk 55 which comprises the steps of treating the silk with aqueous solutions of heavy metal compounds in presence of acid compounds and then transferring the silk directly, without washing, neutralizing or acidifying it, into the following weighting bath.

4. A method of weighting natural silk 60 which comprises the steps of treating the silk with aqueous solutions of heavy metal compounds in presence of acid compounds, squeezing it, and then transferring it di-

rectly, without washing, neutralizing or acidifying it, into an aqueous solution of alkali-metal phosphate.

5. A method of weighting natural silk 70 which comprises the steps of treating the silk with solutions of heavy metal compounds in presence of acid compounds and protective colloids, squeezing it and then transferring it directly, without washing, neutralizing or acidifying it, into an aqueous solution of alkali-metal phosphate.

6. A method of weighting natural silk 75 which comprises the steps of treating the silk with solutions of tin tetrachloride in presence of acid compounds and protective colloids, squeezing it and transferring it directly, without washing, neutralizing or acidifying it, into an aqueous solution of alkali-metal phosphate.

7. A method of weighting natural silk 80 which comprises the step of treating the silk in a single bath containing in aqueous solution a heavy metal compound, an acid compound, and a  $P_2O_5$ -compound.

8. A method of weighting natural silk 85 which comprises the step of treating the silk in a single bath containing tin tetrachloride and phosphoric acid.

9. A method of weighting natural silk 90 which comprises the step of treating the silk in a single bath containing in aqueous solution a heavy metal compound, an acid compound and protective colloids.

10. A method according to claim 3 in 95 which the precipitation treatment of the silk is followed by a treatment with an aqueous solution of alkaline reacting substances.

11. A method according to claim 3 in 100 which the precipitation treatment of the silk is followed by a squeezing and a treatment with an aqueous solution of alkaline reacting substances.

12. A method according to claim 3 in 105 which the precipitation treatment of the silk is followed by a squeezing and a treatment with an aqueous solution of ammonium carbonate.

13. A method of weighting natural silk 110 which comprises the steps of treating the silk with aqueous solutions of heavy metal compounds in presence of organic acids, and precipitating without washing, neutralizing or acidifying the silk, the heavy metal compounds taken up by the silk as compounds insoluble in water.

14. A method of weighting natural silk 115 which comprises the steps of successively treating the silk with an aqueous solution of tin tetrachloride in presence of organic acids, and without washing, neutralizing or acidifying the silk with an aqueous solution of primary sodium phosphate.

In testimony whereof I affix my signature.